# EUROPEAN PATENT SPECIFICATION

(11) **EP 0 936 315 B1**
(45) Date of publication and mention of the grant of the patent: **03.09.2003**
(21) Application number: 98307342.0
(22) Date of filing: 10.09.1998
(51) Int. Cl.: E02D 31/00

(54) **Clay liner**
Ton-Deckschicht
Revêtement en argile

(30) Priority: 13.02.1998 US 23932; 13.08.1998 US 133207
(43) Date of publication of application: 18.08.1999
(73) Proprietor: AMCOL INTERNATIONAL CORPORATION, Arlington Heights, Illinois 60004 (US)
(72) Inventor: McKendrick, Francis Ryan, Winnetka, Illinois 60093 (US)
(74) Representative: W.P. Thompson & Co.

(56) References cited:
- US-A- 3 561 177
- US-A- 5 180 255
- US-A- 5 187 915
- US-A- 5 258 217
- US-A- 5 360 294

## Description

### FIELD OF THE INVENTION

The present invention is directed to an improved, flexible geosynthetic clay liner that is an effective water barrier for ponds, lagoons, waste water containment areas, and for lining concrete surfaces such as concrete plaza decks, concrete foundation walls, and the like. More particularly, the present invention is directed to a geosynthetic clay liner comprising two fabric layers and an intermediate layer of water-swellable clay, such as a sodium montmorillonite clay, wherein the two fabric layers are structurally secured to surround an intermediate layer of clay, in any manner, such as by gluing, compression (U.S. 5,584,609) or by sewing or needle-punching the fabric layers together to confine the clay therebetween. In accordance with the present invention, one of the fabric layers, in contact with the pond or lagoon bed, earthen surface, or foundation wall, includes an open structure that is sufficiently open to permit the extrusion of the clay therethrough when the clay becomes hydrated and swells. The hydrated clay and some water extrudes through the open fabric structure and contacts an adjacent surface that it is applied against, e.g., a pond or lagoon bed, earthen surface, or concrete foundation wall, thereby blocking the lateral migration of water between the adjacent surface, e.g., concrete foundation wall, and the liner to prevent that water from finding a path through the surface to be protected.

### BACKGROUND OF THE INVENTION AND PRIOR ART

The present invention relates to clay geosynthetic liners which are used to form water barriers. The geosynthetic clay liners are useful for lining a surface for protecting that surface against the penetration of water therethrough, particularly for protecting water holding areas, waste water holding areas, concrete surfaces, and the like, such as horizontal plaza decks and vertical concrete foundation walls.

The use of water-swellable smectite clay, such as sodium bentonite, to create a low permeability barrier in landfills and ponds is well known. Bentonite is a clay material that occurs naturally and it expands when hydrated upon absorption of water. When the bentonite absorbs water and expands, it is capable of forming a barrier with low permeability to water migration if the bentonite is properly contained. The geosynthetic clay liners of the present invention rely on incomplete clay containment via extrusion of water-containing, water-swellable clay therethrough upon hydration to prevent the lateral migration of water under the liners.

Geosynthetic clay liners primarily are made with two sheets, e.g., a carrier sheet and a cover sheet, surrounding a layer of water-swellable clay. The primary backing or carrier sheet is normally the more durable material and the liner is often disposed such that the carrier sheet lies against the surface to be protected against water penetration. The cover sheet, also referred to as scrim, is normally less durable than the carrier sheet. The product, including a layer of water-swellable bentonite clay disposed between the two sheets (cover sheet and carrier sheet) is often referred to as a geosynthetic clay liner or GCL.

In order for the water-swellable clay, such as sodium bentonite, to create an effective water barrier, it must be properly contained, such as contained between two sheets - a carrier sheet and a cover sheet. The bentonite may be held in place by glue applied to the carrier sheet; by compression of two sheets surrounding a wet layer of bentonite, e.g., this assignee's U.S. Patent No. 5,584,609, by needle-punching the cover sheet to the carrier sheet; or by stitching the carrier sheet to the cover sheet, or a combination thereof. The sheets may be manufactured from durable woven or non-woven materials or sheets that do not permit the bentonite to migrate through the material.

In accordance with this Assignee's prior U.S. Patent No. 5,350,255, it is known to manufacture a geosynthetic clay liner, for use in landfills, that includes an open structure in the fabric edges for migration of bentonite clay where two geosynthetic clay liners overlap. As indicated in the '255 patent, the open weave is confined to the overlap portions of the GCLs to prevent water penetration in the areas of GCL overlap, and the majority of the GCL has a more closed weave for proper clay confinement in order to maintain the low permeability needed in a landfill environment.

US 5187915 describes a panel, and method of making the panel, useful as a water barrier including an intermediate layer of a water-swellable colloidal clay, such as bentonite, sandwiched between two layers of sheet material, such as paperboard, wherein at least one of the sheet material layers has a plurality of spaced apertures, or water channels, extending from the exterior of the panel to the intermediate water-swellable clay layer. The sheet material layer containing water channels includes a coating of a removable material completely across the water channels in the facing sheet having controlled, predetermined water-solubility so that the intermediate water-swellable clay layer is quickly hydrated after solubilization and removal of the coating material, and to prevent clay hydration during installation, prior to removal of the coating material.

US 5360294 discloses a geosynthetic clay liner provided for installation in landfill sites equipped with lower drainage systems. Overlap extensions disposed on outer edges of the liners effectively contain the activated bentonite.

US 3561177 discloses a laminated building panel for maintaining a water barrier compound in position against a structure which is to be waterproofed including a member providing a plurality of adjacent compartments extending in a plurality of directions, a water barrier compound in each of the compartments, a flexible backing layer covering the rear of said compartments and being water impervious and abrasion resistant, and a flexible facing layer for placement in contiguous relationship with a structure to be waterproofed, the facing layer being porous to permit penetration of water into the compartments for activating the water barrier compound.

In accordance with the prior art, by properly containing the bentonite between two sheets that do not allow for migration of the bentonite, the bentonite has been properly contained and, upon hydration by water, the bentonite will swell and form an effective water barrier. The geosynthetic clay liners of the present invention, on the other hand, provide for controlled migration of water-swellable clay and clay-contained water through an "open" fabric side to prevent lateral migration of water behind the liners.

### SUMMARY OF THE INVENTION

According to the present invention there is provided a composite structure comprising a surface to be protected from water penetration having an inner sheet material layer of a geosynthetic clay liner, said geosynthetic clay liner comprising an inner sheet material layer and an outer sheet material layer having a layer of water-swellable smectite clay disposed therebetween, said inner sheet material layer including a more open structure, across its entire surface, than the outer sheet material layer, and said inner sheet material layer having at least 5% void area, such that upon hydration of said clay, the clay extrudes through the inner sheet material layer, but not through the outer sheet material layer.

Also according to the present invention there is provided a method of protecting a surface against water penetration comprising disposing a geosynthetic clay liner as defined herein, against said surface with the inner sheet material layer disposed against said surface.

The geosynthetic clay liner (GCL) includes a layer of water-swellable smectite clay, e.g., sodium montmorillonite, disposed between a carrier sheet and a cover sheet. An inner sheet, disposed against the surface to be protected against water penetration - either the carrier sheet or the cover sheet - is made of material having a more open structure that allows hydrated bentonite to migrate through it. The other, e.g., outer sheet, includes a more closed structure and, therefore, precludes bentonite migration through it. The GCL can be held together in any manner known, e.g., by adhesively affixing the clay to the sheet material layers, by high pressure compression (45-85 pounds per lineal inch) of the fabrics together surrounding a wet layer of water-swellable clay (e.g., 20-50% by weight water, based on the dry weight of the clay); or by needle-punching or stitching the sheet material layers together surrounding the intermediate clay layer.

Upon hydration, the smectite clay swells to form the barrier. Because the outer sheet or fabric includes a relatively more closed structure than the inner sheet, the bentonite is substantially contained and does not substantially migrate through the outer sheet. Preferably, the outer sheet material layer, when subjected to a pressure of 54.6 psi, does not permit migration of wet clay therethrough more than about 0.01 gm/cm². More preferably less than 0.006 gm/cm² wet clay extrudes through the outer sheet material layer at 54.6 psi. However, because the inner sheet is more open or is more loosely woven, the hydrated bentonite substantially migrates through it in a minimum amount of at least about 0.15 grams (wet basis) per cm², preferably at least about 0.2 grams/cm² when subjected to a pressure of 54.6 pounds per square inch (psi), as described in more detail hereinafter. The extruded, hydrated clay that migrates through the inner sheet engages the adjacent surface to be protected, e.g., a pond or waste water lagoon earthen surface or a concrete foundation wall. The substantial migration of the bentonite through the inner sheet ensures that an effective seal is created, to protect against lateral water movement between the geosynthetic clay liner and the adjacent surface to be protected.

The open structure of the inner fabric sheet may be obtained by employing a looser weave (i.e., lower warp yarn count) than the closed structure of the outer sheet (higher warp yarn count). In particular, it has been found that the surface of the inner sheet should have at least about 5%, preferably at least about 6%, of its surface area as void or open area. If a non-woven geotextile is used as the inner fabric sheet material, the weight of the geotextile, in order to provide at least 5% void or open area in its surface, generally should be in the range of about 100 g/m² to about 200 g/m², preferably about 125 g/m² to about 175 g/m². However, the basis weight can vary substantially both above and below the 100 g/m² to 200 g/m² range, particularly when perforated or slit to provide more clay migration, so long as the hydrated clay extrudes through the open fabric sheet in an amount of at least 0.15 g/cm², preferably at least about 0.2 g/cm² when subjected to a pressure of 54.6 psi. The more open structure of woven inner sheet materials also may be obtained by a perforation or slitting process that creates a structure that will allow for substantial water-swellable clay migration through it.

The method of using a more loosely woven or more open inner sheet (e.g., having a lower warp yarn count) is preferred but the looser weave and the perforation/slitting methods are alternative embodiments that are within the scope of the present invention. The needle-punching and perforation/slitting methods are especially adaptable for geosynthetic clay liners made without gluing the bentonite to one of the sheets (i.e., compression consolidated or a needle-punched liner). The loosely woven and perforated/slitted methods provide the open structure for the inner sheet and the term "open" is meant to indicate sufficient open area for ease of hydrated clay migration through the sheet material in an amount of at least 0.15 g/cm², preferably at least 0.2 g/cm², when subjected to a pressure of 54.6 psi (376.5 kN/m²). Regardless of the percent open area, the inner sheet material layer should extrude at least 0.15 g/cm² of hydrated clay composition (clay and water) when subjected to a pressure of 54.6 psi, preferably at least 0.2 g/cm². In contrast, the term "closed" is meant to indicate a structure that does not permit bentonite migration therethrough in an amount of more than 0.01 gm/cm² at a pressure of 54.6 psi, e.g., a tightly woven sheet material layer.

Accordingly, one aspect of the present invention is to provide a clay liner comprising an inner sheet material layer, an outer sheet material layer, and a layer of water-swellable smectite clay therebetween, wherein said inner sheet material layer includes a more open structure than the outer sheet material layer, such that upon hydration of said clay, the clay extrudes through the inner sheet material layer, but not through the outer sheet material layer, to protect against lateral migration of water between the surface being protected and the outer surface of the inner sheet material layer.

Another aspect of the present invention is to provide a plurality of clay liners that can be disposed against a sloped, vertical, or horizontal surface side-by-side, without overlap, wherein the clay liner includes an open fabric disposed against the surface to be protected against water penetration, such that upon hydration of the clay contained within the liner, the clay will extrude through the open fabric to stop lateral migration of water that penetrates to the protected surface from between adjacent liners.

The above and other aspects and advantages of the present invention will become more apparent from the following detailed description of the preferred embodiments, taken in conjunction with the drawings.

### BRIEF DESCRIPTION OF THE DRAWINGS

FIG. 1 is a perspective view of one embodiment of the clay liner, e.g., geosynthetic clay liner (GCL) of the present invention;
FIG. 2 is a partially broken-away top view showing a plurality of the GCLs of the present invention disposed against a concrete foundation wall or earthen surface applied by overlapping adjacent GCLs;
FIG. 3 is a side view showing a plurality of the GCLs of the present invention disposed on top of a horizontal concrete plaza deck applied side-by-side without overlap;
FIG. 4 is a perspective view of another embodiment of the GCL of the present invention having an "open" side formed by slitting an inner sheet material layer to provide at least 5% open area in the surface of the inner sheet material layer; and
FIG. 5 is a perspective view of a slitting apparatus forming slits in the GCL of FIG. 4.

### DETAILED DESCRIPTION OF THE PREFERRED EMBODIMENTS

Like reference numerals will be used to refer to like or similar parts from Figure to Figure in the following description of the drawings.

FIG. 1 is an illustration of the geosynthetic clay liner 10 including an outer cover sheet 11, a water-swellable smectite clay, e.g., sodium bentonite, layer 12 and an inner carrier sheet 13. All of the Figures and the description below depict the cover sheet as the outer sheet when installed and the carrier sheet as the inner sheet that is disposed against the surface to be protected, when installed.

The outer or cover sheet 11 is more tightly woven or has a more closed structure than the inner or carrier sheet 13. For woven fabrics, the outer or cover sheet 11 has a higher warp count than the warp count of the inner or carrier sheet 13, or the inner sheet 13 is perforated, or slit to include at least 5%, preferably at least about 6%, up to about 25% void or open area in the surface, preferably about 8% to about 20%, more preferably about 10% to about 15% void area in its outer surface. The inner sheet can be woven; non-woven, particularly a non-woven synthetic fiber, such as polypropylene; and/or a polymeric sheet material layer, each of which may be friction enhanced in accordance with this assignee's U.S. Patent No. 5,403,126, hereby incorporated by reference. Nonwoven sheet materials preferably have a weight in the range of about 100 g/m² to about 200 g/m², at a thickness of about 1/32 inch to about 1/8 inch, and provide at least 5% open area, preferably at least about 6% open area, in their outer surface, along the entire outer surface, more preferably about 125 g/m² to about 175 g/m² at a thickness of about 1/32 inch to about 1/8 inch, to provide at least 5% open area along the entire outer surface of the inner sheet material.

Regardless of the percent open area for both the woven and non-woven inner sheet material layers 13, the inner sheet material layer 13 should be sufficiently "open" such that it extrudes at least about 0.15 grams/cm² of hydrated clay (clay plus water) therethrough when subjected to a pressure of 54.6 psi, preferably at least 0.2 grams/cm² of wet clay, most preferably about 0.3 gm/cm² to 0.5 gm/cm². On a dry weight basis, the amount of clay extruded through the open sheet material layer should be at least about 0.03 gm/cm², preferably at least about 0.04 gm/cm², most preferably about 0.05 gm/cm² to about 0.1 gm/cm². The more open inner sheet 13 provides for substantial migration of the bentonite 12 inwardly through the inner sheet 13 upon hydration of the bentonite 12 with water.

An illustration of the installation of the geosynthetic clay liner 10, like the one shown in FIG. 1, is illustrated against a vertical, concrete foundation wall or earthen surface 20 in FIG. 2, and on top of a concrete plaza deck 22 in FIG. 3.

Upon hydration by water, the bentonite layer 12 (preferably about 1/16 inch to about 1/4 inch in thickness) migrates inwardly through the more open inner sheet 13 in an amount of at least about 0.15 gm/cm², preferably at least about 0.2 gm/cm², and engages the surface 20 or 22 to be protected, as illustrated in FIGS. 2 and 3. The expanding and migrating hydrated bentonite composition 12 forms a seal along the surface 20 or 22 to be protected that prevents the lateral migration of water along the surface 20 or 22.

The preferred material for fabrication of the inner or carrier sheets is fabric woven from polypropylene fibers, such as 80-VOL fabric produced by Synthetic Industries, Inc. of Chatanooga, Tennessee, which may be then slit or needle-punched, that extrudes at least 0.15 gm/cm² of hydrated clay composition when subjected to a pressure of 54.6 psi. The carrier and cover sheets have a thickness from, for example, about 1/32 inch to about 1/4 inch, preferably about 1/16 inch to about 1/8 inch, and, to achieve the full advantage of the present invention, the inner sheet 13 has a void area of at least about 8% of the surface area.

As shown in FIG. 4, preferably the inner sheet material layer 13 of the geosynthetic clay liner 10 initially has, or can be provided with, at least 5% void area in its outer surface, by slitting or needle-punching to provide slits or holes 24 completely through the inner sheet material layer 13. The optional slits or holes 24 can be formed prior to applying the inner sheet material layer over the clay layer 12 or, preferably, as shown in FIG. 5, are applied through the inner sheet material layer 13 after construction of the geosynthetic clay liner 10. As shown in FIG. 5, a slitting apparatus 26 includes a rotatable slitting bar 27, that carries a plurality of slitting knives 28, and the slitting bar 27 can be rotated via motor 30 to apply a uniform array of slits 24 that are disposed along the entire outer surface of the inner sheet material 13. The slits 24 preferably provide at least 5% void or open area in the outer surface of inner sheet material layer 13, more preferably about 8% to about 15% void or open area.

In the preferred embodiment of the geosynthetic liner, the inner sheet is a polypropylene woven material, 80-VOL from Synthetic Industries, Inc., that extrudes an average of 0.034 gm/cm² at 54.6 psi compared with earlier product from this Assignee (prior art) that extruded 0.0056 gm/cm² at 54.6 psi.

In order to test the wet clay extrusion or migration through the open sheet material 13 (see FIG. 1) five identical clay liner samples were prepared from pieces of a geosynthetic clay liner having a woven polypropylene sheet material inner layer 13 (80-VOL from Synthetic Industries, Inc.), and a non-woven polypropylene, needle-punched outer sheet material layer 11 (GEOTEX 650 from Synthetic Industries, Inc.) that sandwich a layer of granular sodium bentonite clay 12 therebetween such that the total thickness of the clay liner is 0.8 cm when hydrated and 0.6 cm prior to wetting (as received after manufacture). The samples were immersed in distilled water for 72 hours to completely hydrate the samples.

### PENETROMETER TEST PROCEDURE

(CL-700A Pocket Penetrometer And One Inch Clay Collection Adapter Foot CL-70¹ From The Soiltest Products Division Of ELE International)
A. After the appropriate hydration period, carefully remove the sample from the immersion tub and place onto a flat, level surface.
B. Weigh the clay collection attachment and record. Attach the clay collection attachment (adaptor foot) to the penetrometer and set the penetrometer to 0 psi following the manufacturer's instructions.
C. Place the penetrometer and clay collection attachment (adaptor foot) vertically on top of the specimen at the approximate center of the 0.1 m² (1.0 ft²) square sample. Holding the penetrometer with the clay collection attachment at a right angle to the test specimen, force the entire apparatus (penetrometer and clay collection attachment) into the specimen applying force as necessary. Continue forcing the apparatus into the material until the penetrometer reaches a maximum value (700 psi).
D. Record the reading on the scale of the penetrometer.
E. Carefully pull out the penetrometer and the clay collection attachment, making sure not to displace any of the clay on or in the clay collection attachment. Scrape any clay off the surface of the material within the cross-sectional area of the clay collection attachment that extruded during the testing procedure, but that may not have been collected in the clay collection attachment. Place this displaced clay in the clay collection attachment.
F. Carefully remove the clay collection attachment from the penetrometer and weigh both the extruded clay and the clay collection attachment.
G. Place the clay collection attachment and the collected clay in a drying oven. Dry the samples for the appropriate time. Reweigh the samples to determine the moisture content of the sample during the test procedure.
H. Repeat for a total of five samples.

¹ The Clay Collection Adaptor is the CL-701 Adaptor Foot from Soiltest Division of ELE International having a 11.3 mm diameter hole drilled into the lower material contacting center for collection of clay. A 700 psi reading on penetrometer is 54.6 psi because of the lower contact area that results from the drilled hole.

The amount of clay extruded through the 1 cm² opening in the clay collection adaptor is shown in the data of the following Table 1:

While only a selection of specific embodiments of the present invention has been illustrated and described, it will at once be apparent to those skilled in the art that variations may be made within the scope of the claims. Accordingly, it is intended that the scope of the invention be limited solely by the scope of the hereafter appended claims and not by any specific wording and the foregoing description.

## Claims

1. A composite structure comprising a surface (20, 22) to be protected from water penetration and a geosynthetic clay liner (10), said geosynthetic clay liner (10) comprising an inner sheet material layer (13) disposed against said surface, and an outer sheet material layer (11) having a layer of water-swellable smectite clay (12) disposed therebetween, said inner sheet material layer (13) including a more open structure, across its entire surface, than the outer sheet material layer (11), and said inner sheet material layer (13) having at least 5% void area, such that upon hydration of said clay (12), the clay (12) extrudes through the inner sheet material layer (13), but not through the outer sheet material layer (11).

2. A composite structure as claimed in claim 1, wherein the inner sheet material layer is a woven fabric having a uniformly disposed more open weave that the outer sheet material layer.

3. A composite structure as claimed in claim 2, wherein the inner sheet material layer is a woven fabric having about 8% to about 15% void area, such that the inner sheet material extrudes at least 0.02 gm/cm² at a pressure of 54.6 psi.

4. A composite structure as claimed in claim 1, wherein the inner sheet material layer is a non-woven fabric and is homogeneously more permeable to hydrated clay than the outer sheet material layer.

5. A composite structure as claimed in claim 1, wherein the inner sheet material layer is a polymeric sheet material layer having holes or slits such that at least 5% of its outer surface area is apparent void or open area, such that the inner sheet material extrudes at least 0.015 gm/cm² wetted clay therethrough at a pressure of 54.6 psi.

6. A composite structure as claimed in any one of preceding claims, wherein the outer sheet material layer is a non-woven fabric.

7. A composite structure as claimed in claim 6, wherein the outer sheet material layer is a non-woven fabric that extrudes less than 0.01 gm/cm² of wetted clay therethrough at a pressure of 54.6 psi.

8. A composite structure as claimed in any one of claims 1 to 5, wherein the outer sheet material layer is a water-impermeable polymeric sheet material layer.

9. A composite structure as claimed in claim 8, wherein the water-impermeable polymeric sheet material layer has a friction enhancing material coated, applied or textured on at least a portion of its outer surface.

10. A composite structure as claimed in any of claims 1 to 5, wherein the outer sheet material layer is a woven fabric that extrudes less than 0.01 gm/cm² of wetted clay therethrough at a pressure of 54.6 psi.

11. A composite structure as claimed in claim 1, wherein the inner sheet material layer includes void or open area in its outer surface of at least 6% and extrudes wetted clay therethrough in an amount of at least 0.015 gm/cm², total weight of clay and water, at 54.6 psi, and the outer sheet material has 0-4% void area in its outer surface, and extrudes wetted clay therethrough in an amount of less than 0.01 gm/cm², total weight of clay and water, at 54.6 psi.

12. A composite structure as claimed in claim 1, wherein the inner sheet material layer includes about 8% to about 15% void or open area in its outer surface, such that the inner sheet material layer extrudes wet clay therethrough in an amount of at least 0.015 gm/cm², total weight of clay and water, at a pressure of 54.6 psi.

13. A composite structure as claimed in claim 12, wherein the inner sheet material layer has a weight of about 100 g/m² to about 200 g/m².

14. A composite structure as claimed in claim 13, wherein the inner sheet material layer has a weight of about 125 g/m² to about 175 g/m².

15. A composite structure as claimed in claim 14, wherein the outer sheet material layer has a weight of at least about 220 g/m², such that the outer sheet material layer extrudes less than 0.01 gin/cm² wet clay, total weight of clay and water, at a pressure of 54.6 psi.

16. A composite structure as claimed in any one of claims 1 to 15, wherein the surface to be protected against water penetration is an earthen surface disposed beneath a water-holding area.

17. A composite structure as claimed in any one of claims 1 to 15, wherein the surface to be protected against water penetration is a concrete surface.

18. A composite structure as claimed in claim 17, wherein said surface is a surface of a concrete wall or concrete deck.

19. A method of protecting a surface against water penetration comprising disposing a geosynthetic clay liner as defined in any one of the preceding claims, against said surface, with the inner sheet material layer disposed thereagainst.

20. A method as claimed in claim 19, wherein the surface to be protected is concrete.

21. A method as claimed in claim 20, wherein the surface to be protected is an earthen surface, disposed beneath a water-holding area.

## Patentansprüche

1. Verbundstruktur, umfassend eine vor Wasserpenetration zu schützende Oberfläche (20, 22) und eine geosynthetische Tondichtungsbahn (10), wobei genannte geosynthetische Tondichtungsbahn (10) eine innere Bahnenmateriallage (13) angeordnet gegen genannte Oberfläche und eine äußere Bahnenmaterialiage (11) mit einer Schicht aus wasserquellbarem Smektit-Ton (12) dazwischen angeordnet umfasst, wobei genannte innere Bahnenmateriallage (13) eine offenere Struktur über ihre gesamte Oberfläche als die äußere Bahnenmateriallage (11) einschließt und wobei genannte innere Bahnenmateriallage (13) eine Hohlraumfläche von mindestens 5 % dergestalt aufweist, dass nach Hydratation von genanntem Ton (12) der Ton (12) durch die innere Bahnenmateriallage (13), aber nicht durch die äußere Bahnenmateriallage (11) extrudiert.

2. Verbundstruktur nach Anspruch 1, worin die innere Bahnenmateriallage ein Gewebe ist, das eine gleichmäßig angeordnete offenere Gewebebindung als die äußere Bahnenmateriallage aufweist.

3. Verbundstruktur nach Anspruch 2, worin die innere Bahnenmateriallage ein Gewebe mit einer Hohlraumfläche von ca. 8 % bis ca. 15 % dergestalt ist, dass die innere Bahnenmateriallage bei einem Druck von 54,6 psi mindestens 0,02 g/cm² extrudiert.

4. Verbundstruktur nach Anspruch 1, worin die innere Bahnenmateriallage ein ungewebtes Gewebe ist und für hydratisierten Ton homogen permeabler als die äußere Bahnenmateriallage ist.

5. Verbundstruktur nach Anspruch 1, worin die innere Bahnenmateriallage eine polymere Bahnenmateriallage mit Löchern und Schlitzen dergestalt ist, dass mindestens 5 % ihrer Außenfläche offensichtlich eine Hohlraumfläche oder offene Fläche dergestalt ist, dass das innere Bahnenmaterial bei einem Druck von 54,6 psi mindestens 0,015 g/cm² angefeuchteten Ton dort hindurch extrudiert.

6. Verbundstruktur nach einem der vorangehenden Ansprüche, worin die äußere Bahnenmateriallage ein ungewebtes Gewebe ist.

7. Verbundstruktur nach Anspruch 6, worin die äußere Bahnenmateriallage ein ungewebtes Gewebe ist, das bei einem Druck von 54,6 psi weniger als 0,01 g/cm² angefeuchteten Ton dort hindurch extrudiert.

8. Verbundstruktur nach einem der Ansprüche 1 bis 5, worin die äußere Bahnenmateriallage eine wasserundurchlässige polymere Bahnenmateriallage ist.

9. Verbundstruktur nach Anspruch 8, worin die wasserundurchlässige polymere Bahnenmateriallage ein reibungsförderndes Material auf mindestens einen Anteil ihrer Außenfläche beschichtet, appliziert oder texturiert aufweist.

10. Verbundstruktur nach einem der Ansprüche 1 bis 5, worin die äußere Bahnenmateriallage ein Gewebe ist, das bei einem Druck von 54,6 psi weniger als 0,01 g/cm² angefeuchteten Ton dort hindurch extrudiert.

11. Verbundstruktur nach Anspruch 1, worin die innere Bahnenmateriallage eine Hohlraumfläche oder offene Fläche in ihrer Außenfläche von mindestens 6 % einschießt und angefeuchteten Ton dort hindurch in einer Menge von mindestens 0,015 g/cm², Gesamtgewicht von Ton und Wasser, bei 54,6 psi extrudiert und das äußere Bahnenmaterial in seiner Außenfläche eine Hohlraumfläche von 0-4 % aufweist und angefeuchteten Ton in einer Menge von weniger als 0,01 g/cm², Gesamtgewicht von Ton und Wasser, bei 54,6 psi dort hindurch extrudiert.

12. Verbundstruktur nach Anspruch 1, worin die innere Bahnenmateriallage eine Hohlraumfläche oder offene Fläche von ca. 8 % bis ca. 15 % in ihrer Außenfläche dergestalt aufweist, dass die innere Bahnenmateriallage nassen Ton in einer Menge von mindestens 0,015 g/cm², Gesamtgewicht von Ton und Wasser, bei einem Druck von 54,6 psi dort hindurch extrudiert.

13. Verbundstruktur nach Anspruch 12, worin die innere Bahnenmateriallage ein Gewicht von ca. 100 g/m² bis ca. 200 g/m² aufweist.

14. Verbundstruktur nach Anspruch 13, worin die innere Bahnenmateriallage ein Gewicht von ca. 125 g/m² bis ca. 175 g/m² aufweist.

15. Verbundstruktur nach Anspruch 14, worin die äußere Bahnenmateriallage ein Gewicht von mindestens ca. 220 g/m² dergestalt aufweist, dass die äußere Bahnenmateriallage weniger als 0,01 g/cm² nassen Ton, Gesamtgewicht von Ton und Wasser, bei einem Druck von 54,6 psi extrudiert.

16. Verbundstruktur nach einem der Ansprüche 1 bis 15, worin die gegen Wasserpenetration zu schützende Oberfläche eine Erdoberfläche ist, die unter einer wasserhaltenden Fläche angeordnet ist.

17. Verbundstruktur nach einem der Ansprüche 1 bis 15, worin die gegen Wasserpenetration zu schützende Oberfläche eine Betonoberfläche ist.

18. Verbundstruktur nach Anspruch 17, worin genannte Oberfläche eine Oberfläche einer Betonwand oder eines Betondecks ist.

19. Verfahren zum Schutz einer Oberfläche gegen Wasserpenetration, umfassend das Anordnen einer geosynthetischen Tondichtungsbahn, wie nach einem der vorangehenden Ansprüche definiert, gegen genannte Oberfläche, wobei die innere Bahnenmateriallage dort dagegen angeordnet ist.

20. Verfahren nach Anspruch 19, worin die zu schützende Oberfläche Beton ist.

21. Verfahren nach Anspruch 20, worin die zu schützende Oberfläche eine Erdoberfläche ist, die unter einer wasserhaltenden Fläche angeordnet ist.

## Revendications

1. Structure composite comprenant une surface (20, 22) à protéger de la pénétration de l'eau et un revêtement en argile géosynthétique (10), ledit revêtement en argile géosynthétique (10) comprenant une couche de matériau feuilleté interne (13) disposée contre ladite surface et une couche de matériau feuilleté externe (11) ayant une couche en argile smectique gonflable à l'eau (12) disposée entre celles-ci, ladite couche de matériau feuilleté interne (13) comportant une structure plus ouverte, dans l'ensemble de sa surface, par rapport à celle de la couche de matériau feuilleté externe (11), et ladite couche de matériau feuilleté interne (13) ayant une zone vide d'au moins 5%, de sorte que lors de l'hydratation de ladite argile (12), l'argile (12) s'extrude à travers la couche de matériau feuilleté interne (13), mais non à travers la couche de matériau feuilleté externe (11).

2. Structure composite selon la revendication 1, dans laquelle la couche de matériau feuilleté interne est une étoffe tissée ayant un tissage plus ouvert et disposé uniformément par rapport à la couche de matériau feuilleté externe.

3. Structure composite selon la revendication 2, dans laquelle la couche de matériau feuilleté interne est une étoffe tissée ayant une zone vide allant d'environ 8% à environ 15%, de sorte que le matériau feuilleté interne extrude au moins 0,02 g/cm² à une pression de 54,6 psi.

4. Structure composite selon la revendication 1, dans laquelle la couche de matériau feuilleté interne est une étoffe non tissée et est plus perméable de manière homogène à l'argile hydratée que la couche de matériau feuilleté externe.

5. Structure composite selon la revendication 1, dans laquelle la couche de matériau feuilleté interne est une couche de matériau feuilleté polymère ayant des trous ou des fentes, de sorte qu'au moins 5% de sa surface externe soit une zone apparente, vide ou ouverte, de sorte que le matériau feuilleté interne extrude au moins 0,015 g/cm² d'argile mouillée à travers celle-ci, à une pression de 54,6 psi.

6. Structure composite selon l'une quelconque des revendications précédentes, dans laquelle la couche de matériau feuilleté externe est une étoffe non tissée.

7. Structure composite selon la revendication 6, dans laquelle la couche de matériau feuilleté externe est une étoffe non tissée qui extrude moins de 0,01 g/cm² d'argile mouillée à travers celle-ci à une pression de 54,6 psi.

8. Structure composite selon l'une quelconque des revendications 1 à 5, dans laquelle la couche de matériau feuilleté externe est une couche de matériau feuilleté polymère imperméable à l'eau.

9. Structure composite selon la revendication 8, dans laquelle la couche de matériau feuilleté polymère imperméable à l'eau possède un matériau améliorateur de frottement, qui est revêtu, appliqué ou texturé sur au moins une partie de sa surface externe.

10. Structure composite selon l'une quelconque des revendications 1 à 5, dans laquelle la couche de matériau feuilleté externe est une étoffe tissée qui extrude moins de 0,01 g/cm² d'argile mouillée à travers celle-ci à une pression de 54,6 psi.

11. Structure composite selon la revendication 1, dans laquelle la couche de matériau feuilleté interne comporte une zone vide ou ouverte dans sa surface externe d'au moins 6% et extrude de l'argile mouillée à travers celle-ci en une quantité d'au moins 0,015 g/cm², en poids total d'argile et d'eau, à 54,6 psi, et le matériau feuilleté externe possède de 0 à 4% de zone vide dans sa surface externe, et extrude de l'argile mouillée à travers celle-ci en une quantité inférieure à 0,01 g/cm², en poids total d'argile et d'eau, à 54,6 psi.

12. Structure composite selon la revendication 1, dans laquelle la couche de matériau feuilleté interne comporte d'environ 8% à environ 15% de zone vide ou ouverte dans sa surface externe, de sorte que la couche de matériau feuilleté interne extrude de l'argile mouillée à travers celle-ci en une quantité d'au moins 0,015 g/cm², en poids total d'argile et d'eau, à une pression de 54,6 psi.

13. Structure composite selon la revendication 12, dans laquelle la couche de matériau feuilleté interne a un poids allant d'environ 100 g/m² à environ 200 g/m².

14. Structure composite selon la revendication 13, dans laquelle la couche de matériau feuilleté interne a un poids allant d'environ 125 g/m² à environ 175 g/m².

15. Structure composite selon la revendication 14, dans laquelle la couche de matériau feuilleté externe a un poids d'au moins environ 220 g/m², de sorte que la couche de matériau feuilleté externe extrude moins de 0,01 g/cm² d'argile mouillée, en poids total d'argile et d'eau, à une pression de 54,6 psi.

16. Structure composite selon l'une quelconque des revendications 1 à 15, dans laquelle la surface à protéger contre la pénétration d'eau est une surface terreuse disposée sous une zone de rétention d'eau.

17. Structure composite selon l'une quelconque des revendications 1 à 15, dans laquelle la surface à protéger contre la pénétration d'eau est une surface en béton.

18. Structure composite selon la revendication 17, dans laquelle ladite surface est une surface de mur en béton ou de terrasse en béton.

19. Méthode de protection d'une surface contre la pénétration d'eau, comprenant la disposition d'un revêtement en argile géosynthétique tel que défini selon l'une quelconque des revendications précédentes, contre ladite surface, la couche de matériau feuilleté interne étant disposée contre celle-ci.

20. Méthode selon la revendication 19, dans laquelle la surface à protéger est le béton.

21. Méthode selon la revendication 20, dans laquelle la surface à protéger est une surface terreuse, disposée sous une zone de rétention d'eau.
